

## UNITED STATES PATENT OFFICE

2,068,498

METHOD OF TESTING AND RESTORING THE  
EFFECTIVENESS OF DETERGENT BATHSFranklin H. Mackenzie, Bywood, Pa., assignor to  
American Chemical Paint Company, Ambler,  
Pa., a corporation of DelawareNo Drawing. Application January 12, 1935,  
Serial No. 1,588

## 4. Claims. (Cl. 87—5)

This invention relates to the art of chemical cleaning and particularly to the art of cleaning with alkaline solutions.

The objects of the invention include the provision of a process for testing and restoring the effectiveness of a detergent bath by means of which it is possible to maintain such a bath substantially uniformly in its original condition of effectiveness and to do so at a minimum of expense and waste.

Cleaning solutions, of course, change their character rapidly during use. For example, an alkaline cleaning solution which may contain, originally, a certain concentration of alkaline salts and of soap may be used to clean pressed steel articles which are contaminated with fixed and mineral oil, fatty acids, solid dirt, filings, etc. Such a solution after a period of use in cleaning steel will lose largely its alkalinity while at the same time gaining in soap and emulsified oil content as well as in its content of suspended solid impurities, etc., so that the solution is no longer in good operating condition. Restoration of such a spent bath is a chemical and physical problem of considerable nicety especially where economy of operation and low cost of materials are factors of importance.

Certain crude methods of control have heretofore been employed in an effort to keep such cleansing solutions in proper working order and these methods have ranged from an occasional titration for alkalinity to an occasional measurement of hydrogen-ion concentration and while restoration of these factors to their original value by the addition of alkali may somewhat improve the spent solution yet it does not restore its original detergent effectiveness. Sooner or later the solution degenerates beyond repair and must be entirely discarded and a fresh bath substituted which, of course, is a very wasteful process. Moreover when proceeding in this way the bath is very likely to have been operating over a great part of its life at considerably less than its maximum effectiveness.

Among those skilled in the art, it is recognized that the detergent properties of a solution are dependent upon quite a variety of factors such as the interfacial tension against the work and against the dirt, the colloidal suspending power for solid dirt, the emulsifying power for liquid non-saponifiable grease, the saponifying power for fixed oils, the surface tension, the viscosity, the surface viscosity, etc.

To evaluate these properties in a factory is of course a practical impossibility and even the laboratory has no certain methods for determining some of them. Moreover, even were measurements of all of these properties available for a certain solution, no immediate practical use could be made of the results, because the substances used in making up the original solution do not impart the different measured properties in individually direct ratio but affect them all in varying degrees, i. e., the relative effect of a particular substance is changed by the presence of the other ingredients, whether these were deliberately added or accidentally introduced. For all of these reasons no certain, definite method for correctly treating a detergent solution to maintain it at a predetermined effectiveness has heretofore been found.

The present invention is based on the discovery that the detergent effectiveness of a solution can be maintained substantially constant if certain of its physical properties are maintained at substantially constant values and, as will appear more fully below, the invention is particularly applicable to cleaning solutions which contain an electrolyte, a foaming agent and suspended matter of such a nature as will permit it to settle out when the solution is allowed to stand. These substances may be deliberately added or may come into the bath accidentally or during its operation and as stated above, the invention is particularly applicable to alkaline solutions containing added or accidentally acquired soaps and suspended solid impurities.

Among those properties which I have found it most useful to maintain at substantially constant values in order to maintain the original effectiveness of a detergent bath, are the following: First, its electrical conductivity—second, the longevity of the foam produced following suitable agitation thereof and third, the quantity of suspended matter which settles out when the solution is allowed to stand undisturbed. I have discovered that these three properties are related in some unknown manner to the properties listed above as determining the cleaning effectiveness of a given detergent bath. However, whatever the reason for the result may be, I have discovered that additions of conductive chemical (alkali chemical), of foaming agent previously selected to carry out the cleaning process and of water in sufficient quantities and proportions so as to maintain the conductivity, the foam life, and the suspended solid content

within predetermined limits, will at the same time maintain the cleaning bath at substantially its original effectiveness.

The ingredients of a cleaning solution can be classified into electrolytes, foaming agents, suspended matter, and diluents. Therefore, any excess or deficiency of any ingredient, is immediately made evident by the process of this invention. It is true that each of the properties is affected more or less by each of the ingredients present, and that the solution can only be maintained in perfect condition by making such adjustments as will bring all three properties simultaneously to the predetermined values. Fortunately, however, each added reagent affects one of the determined properties to a much greater extent than it does either of the others. Thus it is possible to adjust the solution to a proper value of each property, by addition of reagent, or by dilution.

For instance, the conductivity is principally affected by the electrolyte concentration; the foam life is affected principally by the content of foaming agent, but also to a considerable extent by electrolyte concentration and content of suspended matter; the suspended matter which settles out in a given time is, of course, chiefly affected by the concentration of such suspended matter in the solution, but also depends on the electrolyte concentration, the content of foaming agent, and the dilution.

It is understood, of course, that the conductivity of the cleaning solution, as of any electrolyte, varies with the temperature of the solution. To be referable to a standard conductivity, any measured conductivity must be made at a standard temperature of the solution; otherwise, it is necessary to know in advance the variation of the conductivity of the solution with temperature and to correct the measured conductivity to the standard temperature before making use of it in correcting the bath compositions. For the purpose of this patent, then, by "electrical conductivity" is meant the numerical value of the electrical conductivity expressed in any absolute or arbitrary units at a standard temperature, whether the conductivity is determined at this standard temperature, or corrected to the standard temperature by appropriate means, when measured at some other temperature.

I will now give a specific example of preferred practice in carrying out my improved method of testing and restoring an aqueous detergent bath.

In one of the cleaning "bowls" of a woolen yarn scouring system of 2,000 gallons capacity, the original solution contained 200 pounds of soda ash and 100 pounds of a special yarn scouring soap which was found by experience to produce satisfactory cleaning of the yarn. The solution which was initially free of suspended matter was kept constantly at a temperature of 130° F.

After operation for approximately a half hour period, the yarn was still emerging in a standard condition with respect to grease content and cleanliness. It was now connected into an alternating current circuit by immersing in it two nickel electrodes each about one inch square which electrodes and an ammeter were coupled at a constant potential of ten volts. The ammeter read .5 ampere.

One hundred cubic centimeters of the solution were then placed in a glass flask bearing indentations which flask was stoppered with a

rubber stopper through which passed a glass rod bearing arms for the purpose of breaking up the solution on shaking and the flask was shaken violently twenty-five times and then allowed to stand until the foam layer had just "broken" leaving a foam-free area on the surface of the solution in the flask. The "life" of the foam was thus determined to be 240 seconds.

Another portion of the solution was placed in a conical graduate holding 200 cc. and the solution allowed to stand undisturbed for approximately five minutes after which time the sediment layer measured 5 cc.

Since, as above stated, the yarn at this time was emerging in satisfactory condition the values just given for conductivity, longevity of foam and sediment volume were adopted as standard.

The scouring process was then continued for approximately one hour more after which the solution was treated as before in order to determine its conductivity, its foam life and its content of suspended matter whereupon the ammeter now read .35 ampere, the foam life was 460 seconds and the volume of sediment 25 was 15 ml. The yarn at this point was now emerging decidedly below standard in quality.

Approximately one-third of the solution was now allowed to run to waste from a bottom outlet in the bowl in order to remove excess suspended matter and the volume was restored with fresh water which was thoroughly mixed in. Similar determinations then resulted in an ammeter reading of .25 ampere, a foam life of 210 seconds, and a sediment volume of 3 cc. Ninety pounds of soda ash were now added and the readings again taken. These were as follows: current 0.50 ampere, foam life 190 seconds, and sediment volume 3 cc.

At this point twenty-five pounds of soap were added following which the same factors were determined whereupon it was found that the current volume again read .5 ampere, that the foam life was 240 seconds and that the sediment volume was 3 cc. Coincidentally the yarn now emerged in standard condition. The described process was continued for upwards of 50 more working hours and during all this time I was enabled to maintain it substantially continuously at or near the standard values for conductivity, foam life and sediment volume and during all this time the yarn emerged in standard condition with respect to grease content and cleanliness.

In connection with the volume of deficient solution which is withdrawn from the bath I desire to explain that this is to be determined very largely by experience but I have found the following to be a reasonably accurate guide. The foam life and the quantity of suspended matter are determined and whichever of these two values is more highly in excess of the desired value is used as an indication of the volume which should be withdrawn so that when this volume is made up by adding water such value will again approximate the desired standard. As stated, with this as an index, experience will soon indicate quite accurately just how much of the spent solution should be replaced with water in order to bring either the foam life or the content of suspended matter (whichever may be the farthest removed from its desired value) back to the value desired.

It will be seen that my improved process may be applied to solutions which may become con-

taminated during use with electrolytes, foaming agents, or suspended matter which can be settled out, as well as to solutions to which these substances have been deliberately added.

5 An example of such an application is in connection with a rinsing solution used to remove alkali, soap, dirt, etc., from yarn which has been scoured in a solution such as has been described above. In such an application, the solution is 10 connected with the electrical conductivity apparatus while the scouring process is in operation. It is agitated with air from time to time, and the foam life determined. It is allowed to stand and the quantity of deposited sediment 15 noted. A quantity of solution is run to waste and fresh water is added to maintain the determined quantities below a predetermined maximum. The indications given by the process will detect imperfect functioning of the "squeeze 20 rolls", etc. When the process is applied to the scouring of raw wool, the wool brings into the first bowl considerable electrolyte. This bowl is initially filled with water only, but gradually accumulates sediment and dissolved salts. By 25 maintaining the conductivity of this solution and its content of sediment within controlled limits by the methods described, the rinsing operation may be kept efficient. Moreover, by this means the quantity of electrolyte carried over 30 with the wool into the first scouring bowl may be closely controlled. In this way the determined conductivities in the scouring bowl are prevented from being irregularly affected by the electrolyte so introduced.

35 In laundries the washing and rinsing solutions may be controlled by this process. Here, however, the solutions are intermittently agitated with air during the washing process by the revolving "wheel". The foam life may be 40 noted by observing the foam on the detergent solution itself.

In certain metal cleaning operations, such as the removal of a light oil coating from full-finished steel panels, the influence of suspended matter is less important than in textile cleaning operations or in the cleaning of material more highly contaminated with solid dirt. In these cases the process may be operated with a less accurate determination of the suspended 45 matter, wasting of the solution to remove suspended matter being necessary only when this exceeds a predetermined limit.

50 Minor variations of the process may suggest themselves to the artisan which do not depart from the spirit of the invention. For instance, agitation of the solution with air may be accomplished by shaking it in a glass flask, by blowing air into it while it is in a working tank, by whipping air into it with rotating paddles, etc. The electrical conductivity of the solution may be determined by any of the means which are well known, such as making the solution between two electrodes one arm of an alternating current bridge circuit; passing a known alternating current through it and noting the potential fall, applying a fixed potential and noting the resulting current, etc. The settleable suspended matter 55 may be determined by allowing the solution to

stand in a graduated vessel and noting the level to which the sediment rises after a given time; or the settled matter may be weighed; or the solution may be caused to flow through a chamber in which its velocity of flow is reduced, and 5 noting the quantity of sediment deposited therein.

I claim:—

1. The method of treating an alkaline cleaning solution containing soda ash and soap in order 10 to maintain it in a condition of maximum effectiveness consisting in determining its electrical conductivity; agitating the solution with air to determine the longevity of the resulting foam; allowing the solution to deposit sediment in order 15 to determine the quantity of suspended matter therein; withdrawing a portion of the solution; and adding soda ash, soap, and water in sufficient quantities to bring the electrical conductivity, the longevity of the foam, and the 20 quantity of settled suspended matter to predetermined values.

2. The method of testing and restoring the effectiveness of an aqueous detergent bath containing an alkaline cleaning chemical and soap, 25 which method comprises the maintenance of substantially constant predetermined standard values for electrical conductivity, foam longevity and content of suspended matter by determining the aforesaid factors and then adding the quantities 30 of alkaline cleaning chemical and soap necessary to bring the conductivity and the foam longevity to their said predetermined values coupled with adjustment of the water content, by withdrawal of a portion of the bath if necessary and replacement thereof with water in 35 order to bring the content of suspended matter also to its said predetermined standard value.

3. The method of testing and restoring the effectiveness of an aqueous detergent bath containing an alkaline cleaning chemical and a foaming agent, which method comprises the maintenance of substantially constant predetermined standard values for electrical conductivity, foam longevity and content of suspended 40 matter by periodically determining said factors and then adding to the bath the quantities of 45 cleaning chemical and foaming agent together with adjustment of the water content necessary to bring the conductivity, the foam longevity and 50 the content of suspended matter to said predetermined standard values.

4. The method of treating an aqueous cleaning chemical and a foaming agent in order to maintain it in a condition of maximum effectiveness, 55 which method consists in determining its electrical conductivity; agitating the bath with air to determine the longevity of the resulting foam; allowing the bath to deposit sediment in order to determine the quantity of suspended matter 60 therein; withdrawing a portion of the bath and then adding water, cleaning chemical and foaming agent in sufficient quantities to bring the electrical conductivity, the longevity of the foam, and the quantity of settled suspended matter at 65 predetermined substantially constant values.

FRANKLIN H. MACKENZIE.